

A. M. STOLTEY.  
EXPANDED WOOD LAMINA.  
APPLICATION FILED OCT. 18, 1909.

974,536.

Patented Nov. 1, 1910.

Fig. 1.



Fig. 2.



Fig. 3.



Inventor

A. M. Stoltey

By Woodgrain & Chandler.

Attorneys

Witnesses

E. Hurst.

M. L. Low.

# UNITED STATES PATENT OFFICE.

ALBERT M. STOLTEY, OF NEWARK, NEW JERSEY.

## EXPANDED-WOOD LAMINA.

974,536.

Specification of Letters Patent.

Patented Nov. 1, 1910.

Application filed October 18, 1909. Serial No. 523,171.

To all whom it may concern:

Be it known that I, ALBERT M. STOLTEY, a citizen of the United States, residing at Newark, in the county of Essex and State 5 of New Jersey, have invented certain new and useful Improvements in Expanded-Wood Laminæ, of which the following is a specification.

This invention relates to a new and useful 10 article of manufacture.

The object of my invention is to provide a new article of manufacture, comprising a laminated body, made up of a plurality of sheets of wood veneer each sheet being 15 provided with a series of parallel extending weakening grooves running lengthwise of the grain, the sheets then being lengthened to tear the same apart within the grooves to provide a wooden openwork, the ungrooved 20 portions being held together by the intervening wood fibers, two or more such torn and lengthened sheets being securely united so that the grain of one sheet will run crosswise to that of the other.

25 A further object of my invention is to provide a laminated body, made up of a plurality of sheets having a flat and a grooved surface the sheets being lengthened to tear the same apart within the grooves, 30 two or more such lengthened sheets being securely united with their flat surfaces in juxtaposition.

35 A still further object is to provide a laminated body comprising a sheet of wood veneer provided with a series of parallel extending weakening grooves running approximately lengthwise of the grain, the sheet being lengthened and torn asunder to provide a wooden openwork, the sheet then 40 being backed with a suitable paper fabric or other covering.

45 A still further object of my invention is to provide a new article of manufacture including two sheets of wood veneer each having a flat and a grooved surface, said sheets being lengthened and torn to provide a wooden openwork said sheets being securely united with their grains running at right angles and facing this lamina with a suitable 50 paper, fabric or other coverings.

With the above and other objects in view the present invention consists in the combination and arrangement of parts as will be hereinafter more fully described and particularly pointed out in the appended claims,

it being understood that changes in the specific structure shown and described may be made within the scope of the claims without departing from the spirit of the invention.

60 In the drawings forming a part of this specification, and in which like numerals of reference indicate similar parts in the several views, Figure 1 shows an enlarged end view of a sheet of grooved wood veneer as used in my invention previous to lengthening the same. Fig. 2 shows a fragmentary portion of a lengthened sheet in top view disclosing the location of the unbroken stay portions of the treated veneer sheet. 65 Fig. 3 shows a lamina made up of two connected lengthened sheets, faced with a covering upon both sides.

70 In carrying out the aim of my invention, I employ a sheet or section 1 of wood veneer and provide one of the faces with a plurality of weakening parallel running grooves 2 the grooves being formed by compressing the wood. This construction then provides a member having the parallel stay 75 forming wood sections 3 with the intervening compressed portions 5. These weakening grooves 2, may run lengthwise of the grain, or they may run slightly oblique to the grain. After the veneer sheets have 80 been grooved, they are lengthened under force, resulting in the sheets separating at the points marking the weakest parts of the woods within the grooves 2. The stay forming portions 3 remain intact, but the compressed wood fibers within the grooves partly 85 separate to provide a wooden openwork as disclosed in Fig. 2. Two or more sheets are then connected in their lengthened condition in such a manner that the 90 stay forming members 3 upon one side of the lamina will run or extend at right angles or obliquely to those upon the opposite side. By this method I provide a lamina, but half 95 the weight of the board of equal thickness, in which the transverse and longitudinal resistance will be greater and which will be 100 flexible. These made up boards or sheets, may be used in the manufacture of receptacles, boxes, mailing boards, covers of 105 books and other articles.

105 The method of grooving and lengthening the veneer may be effected in any suitable workman like manner.

110 From the foregoing it will be seen that I

provide an expanded wood veneer, and that a plurality of such expanded veneers are securely united to form a laminated board. This process includes the forming of 5 strips of veneer running transversely of the wood grain, by suitable planing means preferably including a lathe for turning a log or block in a plane transverse of the grain and a planing member movable transversely 10 of the lathe to engage the periphery of the log or block constantly to produce a continuous strip of veneer. The veneer may then be moistened or treated in any other suitable manner to adapt the fiber of the 15 wood to ready separation without breakage. It then may be lengthened by being passed between two sets of rollers, the second set engaging the veneer moving at a greater surface speed than the first set. The first 20 set of rollers should have smooth surfaces, as should one of those in the second set; but the other roller in the second set should be provided with longitudinally extending 25 ribs, which compressing the wood slightly against the smooth roller weakens the structure of the veneer just enough to allow the spreading of the fibers on the line of compression.

And having thus described my said invention what I claim as new and desire to secure by United States Letters Patent is:

1. As a new article of manufacture, an expanded wood veneer comprising a wooden openwork held together by intact portions 35 of wood.

2. As a new article of manufacture, an expanded wood veneer comprising a wood openwork held together by unaffected portions of wood running lengthwise of the 40 grain.

3. As a new article of manufacture, an expanded wood veneer comprising a wood openwork held together by un torn portions of wood running diagonally.

4. As a new article of manufacture, a wood veneer having parallel running grooves the wood fiber within the grooves being partly separated.

5. As a new article of manufacture a 50 wood veneer provided with a parallel running series of grooves formed by compressing the material, the wood fibers within the grooves being separated.

6. As a new article of manufacture a 55 laminated body made up of a plurality of

sheets of wood veneer each sheet being expanded to provide a wood openwork held together by unaffected portions of wood said sheets united with their grains extending and running at an angle.

60

7. A laminated body made up of a plurality of sheets of wood veneer stretched to provide break joints in the wood to form a flat openwork.

8. As a new article of manufacture a 65 wood veneer provided with parallel running weakening grooves, the wood fibers within the grooves being separated, and a backing covering said veneer.

9. A laminated body, made up of a plurality of sections of wood veneer, each section having a series of parallel running stay forming portions, the wood fibers between said stay forming portions being separated, said veneer sections being secured to one another.

10. A laminated body made up of a plurality of sections of wood veneer, each section having a series of parallel running stay forming portions, the wood fibers between 80 said stay forming portions being separated, said veneer sections being secured to one another, and a facing covering said veneer sections.

11. As a new article of manufacture a 85 wood veneer having a series of parallel running stay forming portions the wood fibers between said stay forming portions being separated.

12. As a new article of manufacture an 90 expanded wood veneer comprising a plurality of parallel running portions of wood, the material between the parallel portions being separated to provide a wood openwork.

95

13. A laminated body comprising a sheet of wood stretched diagonally to separate its fibers, and a second similarly stretched sheet of wood disposed with the major dimensions of its fibers at right angles to those of the 100 first named sheet.

14. As a new article of manufacture, a sheet of wood stretched laterally and diagonally of its grain to separate its fibers.

In testimony whereof I affix my signature, 105 in presence of two witnesses.

ALBERT M. STOLTEY.

Witnesses:

WILLIAM CRAWFORD,  
JOHN W. JORALEMON.